

1,404,267.

F. H. BULLINGER,  
RESISTANCE UNIT AND METHOD OF MAKING,  
APPLICATION FILED APR. 27, 1920.

Patented Jan. 24, 1922.

Fig:1.



Fig:3.



Frederic H. Bullinger Inventor  
By his Attorneys  
Edwards, Sager & Power.

# UNITED STATES PATENT OFFICE.

FREDERIC H. BULLINGER, OF YONKERS, NEW YORK, ASSIGNOR TO WARD LEONARD ELECTRIC COMPANY, A CORPORATION OF NEW YORK.

## RESISTANCE UNIT AND METHOD OF MAKING.

1,404,267.

Specification of Letters Patent. Patented Jan. 24, 1922.

Application filed April 27, 1920. Serial No. 377,012.

To all whom it may concern:

Be it known that I, FREDERIC H. BULLINGER, a citizen of the United States, residing at Yonkers, in the county of Westchester and State of New York, have invented certain new and useful Improvements in Resistance Units and Methods of Making, of which the following is a specification.

This invention relates to resistance units or rheostatic units, in which the resistance element or elements are imbedded in or covered by an insulating coating, such as vitreous enamel, or other coating, which is fused or baked in a furnace of comparatively high temperature.

In resistance units of this character, it is often desired to provide rigid terminal connections which form a part of the unit when completed, in order to afford convenient contacts or terminals for the connection of external leads.

The main object of this invention is to provide an improved construction of the unit and method of making, which will insure good electrical contact of such terminals with the resistive conductor of the unit, and to accomplish this in a manner which will simplify the cost of manufacture, especially in the cost of labor.

Devices of this character present a difficult problem in making connection between the terminal and the resistive conductor. This is due to the comparatively high temperature of the furnace in baking or fusing the insulating coating, which high temperature causes oxidation of the metals where they make contact and give a poor electrical connection or none at all in the completed article, unless special means are taken to insure the connection. One method heretofore employed is to place a metal clip over the connection between the resistive conductor and the terminal and hammer the parts together which gives such intimate contact that the air is excluded between the contacts and oxidation avoided. But this method requires a considerable amount of hand labor, especially where one or more interior taps are provided, as the maker must interrupt the winding of the resistive conductor to make the tap connection before continuing with the winding.

By my present invention, the winding of the resistive conductor may be proceeded

with continuously and the taps applied afterwards which saves considerable time. Also I secure a good soldered joint between the resistive conductor and the terminal which is of a character that is not destroyed in the firing of the unit, and I further cause the operation of baking or fusing the insulating coating to also make the soldered joint. I am furthermore enabled to locate the soldered joint under the terminal or tap connection where it is not only effectively soldered but insures a protected permanent connection.

The accompanying drawings illustrate one form of unit embodying and made in accordance with my invention, Fig. 1 being a side elevation without the insulating coating applied and with parts broken away; Fig. 2 an end view of Fig. 1; and Fig. 3 a side elevation of the unit complete.

In this instance a tube 1 of earthenware, porcelain or like material is wound with the resistive wire 2. The terminals or tap connections are shown at 3 and in this example consists of a copper band clamped over the tube and resistive conductor and firmly held by a terminal screw 4 and nut 5, the screw passing through holes in the extensions 3' of the band 3. Additional nuts and washers 6 are provided on screw 4 for making external connections to the taps without disturbing or loosening the bands, or any other suitable auxiliary means may be provided for making external connections, such as prolonging the extensions 3 for receiving additional terminal screws.

Before clamping the bands in place, I introduce a piece or sheet of solder 7 under each band and between it and the resistive conductor together with a suitable flux. This solder should have a fusing point approaching or comparatively near the furnace temperature required to fuse or bake the enamel coating. When the bands are clamped in place with the solder applied as above stated, it gives a firm contact of the solder with the bands and resistive conductor. The insulating coating 8 of enamel or other suitable material is then applied to cover the resistive conductor and to cover wholly, or partially, the bands 3. The unit is then fired or baked at the required temperature to fuse or bake the insulating coating, which operation also fuses the solder

to give a soldered connection and a good permanent joint and electric connection between the conductor and taps.

In order to secure satisfactory results by this method, it is important that the solder used shall have a fusing point approaching or comparatively near the temperature to which the insulating coating is subjected in baking or fusing it. In the case of fusing 10 a vitreous enamel insulating coating, the temperature to which the unit is commonly subjected in firing is from 600 to 700 degrees centigrade. If the usual solders, which have a low fusing point, be used in such a case, 15 even when soldered before firing or attempted to be soldered during firing, the high temperature of firing will cause such solder to become very thin and run away from between the conductor and taps and spoil the 20 soldered joint. It also causes the adjoining parts of the joint to become oxidized and prevents an electrical connection or permits such a poor one as to be unsatisfactory or lacking in permanence. By using a solder 25 which has a high fusing point and which approaches the firing temperature, the soldering may be accomplished during the firing; because at the high temperature of firing, the solder softens or melts sufficiently to 30 make a good soldered joint and maintains it during firing because it does not become so thin as to run and spoil the soldered joint or have the parts exposed to oxidation. I have obtained satisfactory results with a

solder composed of about 80 per cent tin 35 and 20 per cent copper which fuses well above 500 degrees centigrade; but other solder alloys may be used having a comparatively high fusing temperature and comparatively near the firing temperature, or 40 not greatly below it.

When I refer to taps in the appended claims, it will be understood that it includes end connections as well as interior connections to the resistive conductor; and where 45 the term enamel is used, it includes any equivalent insulating coating.

Although I have described a preferred embodiment and method of my invention, this may be modified without departing 50 from the scope thereof.

I claim:—

1. The method of making a resistance unit which consists in applying the resistive conductor to a support, placing a tap in connection with the conductor with solder interposed, applying a coating of enamel material thereto, and heating the unit to simultaneously fuse the solder and enamel. 55

2. The method of making a resistance unit 60 which consists in applying the resistive conductor to a support, clamping a tap against the conductor with solder interposed, said solder having a high fusing point, applying a coating of enamel material thereto, and heating the unit to simultaneously fuse the solder and enamel. 65

FREDERIC H. BULLINGER.